# EUROPEAN PATENT SPECIFICATION

(11) **EP 0 066 656 B1**
(45) Date of publication and mention of the grant of the patent: **25.09.1985**
(21) Application number: 81302442.9
(22) Date of filing: 02.06.1981
(51) Int. Cl.: C23C 18/34, C03C 17/10

(54) **Process for preparing nickel layer**
Verfahren zur Herstellung einer Nickelschicht
Procédé pour la préparation d'une couche de nickel

(43) Date of publication of application: 15.12.1982
(73) Proprietor: ASAHI GLASS COMPANY LTD., Chiyoda-ku, Tokyo (JP)
(72) Inventor: Kobayashi, Takayuki, Yokohama-shi Kanagawa-ken (JP); Tamamura, Ryo, Yokohama-shi Kanagawa-ken (JP)
(74) Representative: Warden, John Christopher

## Description

### Background of the invention

### Field of the invention

The present invention relates to a process for preparing a nickel containing layer by a chemical plating.

### Description of the prior arts

Glass plates having each thin transparent or translucent metal layer made of silver, nickel or aluminum which reflect or intercept heat radiation of solar or radiant heat have been known as heat radiation reflecting glass plates and have been used as a single glass plate, a double layer glass plate or a laminated glass plate in buildings, vehicles and various apparatuses and instruments. Among these metal coated glass plates, the glass plates having a nickel layer has superior heat radiation reflectivity and superior durability to the glass plates having the other metal layer and has a transparent neutral grey color and accordingly, it is one of excellent heat radiation reflecting glass. The nickel layer of said glass plate is usually formed by a vacuum evaporation process, a sputtering process, or a chemical plating process. Among them, the chemical plating process for applying a nickel salt and a reducing agent on a glass plate and reducing said nickel salt by a chemical reaction to form a nickel layer on the glass plate has various advantages that the nickel layer can be formed at an ambient temperature, and it can be formed for a short time in high productivity and it can be easily formed without using an expensive apparatus as required in the vacuum evaporation process or the sputtering process. The chemical plating process, however, has disadvantages that a rate of deposition is not easily controlled and a nickel layer having a desired thickness or uniform thickness is not easily formed and color uneveness is caused, and pinholes are caused and a uniform dense layer is not easily formed.

### Summary of the invention

It is an object of the present invention to provide a process for preparing a nickel containing layer having excellent characteristics without the above-mentioned disadvantages by a chemical plating process.

According to the invention there is provided a process for depositing a nickel containing layer on a substrate, in which the substrate is treated with a nickel salt and a reducing agent for reducing said nickel salt, characterized in that said treatment is carried out in the presence of diethylenetriamine and/or imidazole.

Preferably the nickel salt and reducing agents are applied successively in separate solutions and the diethylenetriamine and/or imidazole is present in the nickel salt solution in a concentration of 1 to 1000 ppm.

Preferably the diethylenetriamine or imidazole is utilised in an amount of 0.02 to 20 wt% based on the nickel salt.

### Detailed description of the preferred embodiments

A substrate made of glass, plastic or ceramic etc. is usually treated by a sensitizing treatment or an activating treatment before the chemical plating process of the present invention. The typical treatment is a treatment for contacting the substrate with an aqueous solution of a stannous salt after water washing and further contacting it with an aqueous solution of a palladium salt.

The typical process for preparing a nickel layer on the substrate is a process for spraying or coating a chemical nickel plating solution comprising a nickel salt and a reducing agent and if necessary, the other additive such as a chelating agent, a pH buffering agent, a pH modifier, a stabilizer etc. on the substrate and forming the nickel layer on the substrate by a chemical reduction or a process for spraying both of a nickel plating solution comprising a nickel salt and if necessary the other additive such as a chelating agent, pH buffering agent, a pH modifier etc. and a solution comprising a reducing agent and a stabilizer on a glass surface and forming a nickel layer on the substrate by a chemical reduction.

The nickel salts used in the process of the present invention can be inorganic or organic water soluble nickel salts such as nickel chloride, nickel sulfate, nickel acetate, nickel bromide, nickel iodide or a mixture of at least two nickel salts. The nickel salt is usually used in a form of an aqueous solution. It is also possible to use the nickel salt in a form of an organic solvent solution or a solution of an organic solvent with water.

In the solution of a nickel salt, it is possible to incorporate a pH modifier which results in an alkaline condition and a chelating agent such as Rochelle salt, EDTA, sodium citrate and sodium gluconate, and a pH buffering agent such as malic acid and/or boric acid so as to easily perform the chemical reduction.

The typical reducing agents can be sodium borohydride, potassium borohydride, formaldehyde, sodium hypophosphite, hydrazine, hydrazinium sulfate, glyoxal, dimethylamine borazane, hydrosulfite, diethyl borazane or a mixture of at least two reducing agents with a stabilizer.

A concentration of a nickel salt in an aqueous solution of a nickel salt used in the process of the present invention is preferably in a range of about 0.1 to 10%.

In the process of the present invention, diethylenetriamine, imidazole or a mixture thereof is present during the chemical reduction of the nickel salt.

The diethylenetriamine and/or imidazole may be incorporated as an additive in a solution of a nickel salt, a solution of a reducing agent, or in a nickel plating solution containing both of a nickel salt and a reducing agent. Alternatively, the diethylenetriamine, and/or imidazole may be applied separately during the chemical reduction process to deposit the nickel layer.

When diethylenetriamine, and/or imidazole is incorporated in the chemical reduction of the nickel salt, a nickel layer having high density, and a uniform thickness without pinhole can be formed. The reason is not clear, however, it is considered to result fine nickel grains deposited by the chemical reduction. Diethylenetriamine imparts especially superior effect.

A time for plating in the deposition of the nickel layer by the chemical plating process is usually in a range of 30 seconds to 10 minutes preferably about 1 minute to 5 minutes.

Atemperature of the solution of a nickel salt, the solution of a reducing agent or the solution of a nickel salt and a reducing salt in the deposition of the nickel layer by the chemical plating process is usually in a range of 10°C to 60°C especially about 30°C. The rate of nickel deposition is varied depending upon the temperature in the chemical plating whereby it is important to maintain the temperature in the chemical plating in constant such as in a range of ±3'C so as to prevent unevenness of color. A temperature of the substrate in the chemical plating is usually in a range of 10 to 60°C preferably about room temperature.

A thickness of the nickel layer formed in the process of the present invention can be selected to be transparent or translucent and to give desired optical characteristics such as desired heat radiation reflectivity and transmissivity etc. and is preferably in a range of 100 to 1000 A. A composition a flow rate of the plating solution, a plating time and a temperature are selected so as to give a desired thickness of the nickel layer.

In the preparation of the nickel layer of the present invention, it is possible to form a composite layer of nickel and an other metal by incorporating a salt of the other metal such as copper, cobalt, iron, silver, gold and platinum together with the nickel salt.

The present invention will be further illustrated by certain examples and references which are provided for purposes of illustration only and are not intended to be limiting the present invention.

### Example 1

A glass plate (300 mmx300 mmx5 mm) was polished with ceria and rinsed with water. An aqueous solution of stannous chloride (SnC12. 2H₂0:1 g/1 liter of water) was sprayed on the surface of the glass plate to perform a sensitizing treatment for 30 seconds and then, the glass plate was rinsed with water and an aqueous solution of palladium chloride (PdC12. nH₂0:0.05 g/1 liter of water; 1.0 ml of 35% HCI/1 liter of water) was sprayed on the surface of the glass plate to perform an activating treatment for 30 seconds and then, the glass was rinsed with deionized water.

The following aqueous solution of the nickel salt and the solution of the reducing agent (30°C) were respectively sprayed on the treated surface of the glass plate at 30°C by each spray-gun at each rate of 0.64 liter/minute and they were kept for 2 minutes to deposit a nickel layer on the glass plate.

The resulting nickel layer formed on the glass plate had a thickness of 500 A and was a dense uniform layer without any pinhole and had uniform color distribution shown by the curve (a) in Figure 1 as visible transmissivity Tᵥ in the longidutinal direction of the glass plate having nickel layer.

The optical characteristics of the glass plate are shown in Table 1.

### Example 2

A glass plate (300 mmx300 mmx5 mm) was polished with ceria and rinsed with water. An aqueous solution of stannous chloride (SnCl₂ · 2H₂O:1 g./1 liter of water) was sprayed on the surface of the glass plate to perform a sensitizing treatment for 30 seconds and then, the glass plate was rinsed with water and an aqueous solution of palladium chloride (PdCl₂ · nH₂O:0.05 g./1 liter of water;,1.0 ml of 35% HCI/1 liter of water) was sprayed on the surface of the glass plate to perform an activating treatment for 30 seconds and then, the glass plate was rinsed with deionized water.

The following aqueous solution of the nickel salt and the solution of the reducing agent (30°C) were respectively sprayed on the treated surface of the glass plate at 30°C by each spray-gun at each rate of 0.64 liter/min. and they were kept for 2 minutes to deposit a nickel layer on the glass plate.

The resulting nickel layer formed on the glass plate had a thickness of 500 Å and was a dense uniform layer without any pinhole and had uniform color distribution shown by the curve (b) in Figure 1.

The optical characteristics of the glass plate are shown in Table 1.

### Reference

In accordance with the process of Example 1 except that diethylenetriamine was eliminated from the aqueous solution of the nickel salt, a nickel layer was formed on the surface of the glass plate.

The resulting nickel layer formed on the glass plate had a thickness of 700 Å and had color distribution shown by the curve (c) in Figure 1.

The optical characteristics were respectively measured under the light incidence from each nickel layer of each sample of glass plate having a thickness of 5 mm.

Figure 1 shows color distributions of nickel layers of the samples.

As it is shown in Table 1 and Figure 1, the nickel layer having the uniform color distribution and less pinhole can be obtained in accordance with the process of the present invention.

## Claims

1. A process for depositing a nickel containing layer on a substrate, in which the substrate is treated with a nickel salt and a reducing agent for reducing said nickel salt, characterized in that said treatment is carried out in the presence of diethylenetriamine and/or imidazole.

2. A process according to claim 1 wherein the nickel salt and reducing agents are applied successively in separate solutions and the diethylenetriamine and/or imidazole is present in the nickel salt solution in a concentration of 1 to 1000 ppm.

3. A process according to claim 1 or claim 2 wherein the diethylenetriamine or imidazole is utilised in an amount of 0.02 to 20 wt% based on the nickel salt.

## Patentansprüche

1. Verfahren zur Abscheidung einer nickelhaltigen Schicht auf einem Substrat, wobei das Substrat behandelt wird mit einem Nickelsalz und einem Reduktionsmittel zur Reduzierung des Nickelsalzes, dadurch gekennzeichnet, daß die Behandlung durchgeführt wird in Gegenwart von Diäthylentriamin und/oder Imidazol.

2. Verfahren nach Anspruch 1, wobei das Nickelsalz und Reduktionsmittel aufeinander folgend in gesonderten Lösungen appliziert werden und das Diäthylentriamin und/oder Imidazol in der Nickels alz-Lösung in einer Konzentration von 1 bis 1000 ppm vorliegt.

3. Verfahren nach Anspruch 1 oder Anspruch 2, wobei man das Diäthylentriamin oder Imidazol in einer Menge von 0,02 bis 20 Gew.-%, bezogen auf das Nickelsalz, anwendet.

## Revendications

1. Procédé pour déposer une couche contenant du nickel sur un support, dans lequel le support est traité avec un sel de nickel et un agent réducteur pour réduire ledit sel de nickel, caractérisé en ce que ledit traitement est effectué en présence de diéthylènetriamine et/ou d'imidazole.

2. Procédé selon la revendication 1 dans lequel le sel de nickel et les agents réducteurs sont successivement appliqués en solutions distinctes et la diéthylènetriamine et/ou l'imidazole sont présents dans la solution de sel de nickel à une concentration de 1 à 1000 ppm.

3. Procédé selon la revendication 1 ou selon la revendication 2 dans lequel la diéthylènetriamine ou l'imidazole est utilisé en une quantité de 0,02 à 20% en poids par rapport au sel de nickel.
